

No. 695,376.

Patented Mar. 11, 1902.

G. G. CONVERS & A. B. DE SAULLES.

PRODUCTION OF ZINC DUST.

(Application filed Sept. 14, 1898.)

(No Model.)

4 Sheets—Sheet 1.

Fig. 1.



Witnesses.

D. W. Edelin.

J. E. Hutchinson Jr.

Inventors.

Geo. G. Convers,  
Arthur B. deSaulles,  
by license of Goldsborough,  
Attns

No. 695,376.

Patented Mar. 11, 1902.

G. G. CONVERS & A. B. DE SAULLES.  
PRODUCTION OF ZINC DUST.

(Application filed Sept. 14, 1898.)

(No Model.)

4 Sheets—Sheet 2.



Fig. 5.



Fig. 3.



Fig. 4.



Witnesses:

D. W. Edelin.

J. E. Hutchinson Jr.

Inventors:  
Geo. G. Convers,  
by Arthur B. de Saulles  
Jennie Goldsbrough  
Attest

No. 695,376.

Patented Mar. 11, 1902.

G. G. CONVERS & A. B. DE SAULLES.

PRODUCTION OF ZINC DUST.

(Application filed Sept. 14, 1898.)

(No Model.)

4 Sheets—Sheet 3.

Fig. 8.



Witnesses:

D. D. Edelin.

J. E. Hutchinson Jr.

Inventors.

Geo. G. Convers,  
Arthur B. de Saulles,  
by Lemire & Goldsborough  
Attny.

No. 695,376.

Patented Mar. 11, 1902.

G. G. CONVERS & A. B. DE SAULLES.

PRODUCTION OF ZINC DUST.

(Application filed Sept. 14, 1898.)

(No Model.)

4 Sheets—Sheet 4.

Fig. 9.



Witnesses:

O. D. Edelji.  
J. E. Hutchinson Jr.

Inventors:  
Geo. G. Convers,  
Arthur B. De Saulles,  
by Lemuel Goldbloway,  
Atty's.

# UNITED STATES PATENT OFFICE.

GEORGE G. CONVERS AND ARTHUR B. DE SAULLES, OF SOUTH BETHLEHEM, PENNSYLVANIA.

## PRODUCTION OF ZINC-DUST.

SPECIFICATION forming part of Letters Patent No. 695,376, dated March 11, 1902.

Application filed September 14, 1898. Serial No. 690,911. (No specimens.)

*To all whom it may concern:*

Be it known that we, GEORGE G. CONVERS and ARTHUR B. DE SAULLES, citizens of the United States, residing in South Bethlehem, 5 in the county of Northampton and State of Pennsylvania, have invented certain new and useful Improvements in the Production of Zinc-Dust; and we do hereby declare the following to be a full, clear, and exact description of the invention, such as will enable others skilled in the art to which it appertains to make and use the same.

Our invention relates to the production from zinc-bearing material of metallic zinc in 15 the finely-divided or granular condition, known as "zinc-dust" or "blue powder." Heretofore, so far as we are aware, this product has been obtained in relatively limited quantities as an auxiliary product in the metallurgy of zinc, whereas the purpose of our 20 invention is to recover substantially the entire zinc component of the retort charge as zinc-dust.

The salient or main characteristic feature 25 of our improvement depends upon the discovery that the zinc-vapors in order to be precipitated in their entirety as zinc-dust should pass at once into a collecting-chamber sufficiently ample to receive them all, care being 30 taken that the pipe or connection through which the vapors are discharged into the collector shall be above the distilling-point of the metal. At the beginning of the operation, when the retort contains a quantity of 35 air, and toward the end of the operation, when the retort-charge becomes lean in zinc, more or less zinc oxid is produced, which oxid is taken off separately, so that it may not mix with the zinc-dust.

40 In the accompanying drawings, Figure 1 represents, partly in section and partly in elevation, a portion of a furnace suitable for the practice of our invention: Fig. 2 represents a cross-sectional view with one of the 45 collectors in place. Fig. 3 represents said collector in front elevation and on a somewhat larger scale. Fig. 4 represents a cross-sectional view of the collector. Fig. 5 represents a rear elevation thereof. Fig. 6 represents a top plan view of the collector-cover. Fig. 7 represents a side elevation thereof.

Fig. 8 represents, partly in section and partly in elevation, another form of furnace suitable for the practice of our invention. Fig. 9 represents a vertical sectional view thereof. 55

Similar letters of reference indicate similar parts throughout the several views.

Referring to the first form of apparatus, (illustrated in Figs. 1 to 7, inclusive,) A indicates the basal portion of the furnace, having the fuel-chamber *a*, grate-bars *b*, ash-pit *c*, and bridge-wall *d*, over which the products of combustion pass to the downtake chimney-flue *e*, as will be readily understood. Upon the side walls of the fuel-chamber rest the 60 open-ended "cannon" *f*, and above them are located the zinc-distilling retorts *n*, the function of the cannon being to distribute the products of combustion about the sides of the retorts and to prevent the retort-bottoms 65 from being subjected to too high a heat. The retorts *n*, as shown, rest upon refractory tiles or bricks built up from the base *A* of the furnace. Above the retort-chamber is provided 70 with the arch *B*, and the entire furnace is 75 strengthened and bonded by buck-stays and cross-ties, as shown. The retorts *n* have each an exit-opening *m* for the zinc-vapors and are charged from the opposite end, which is 80 shown in Fig. 2 as luted up. The corresponding wall of the furnace is removable in order to obtain access to the retorts and cannons. 85 Adjacent to the vapor-exit ends of the retorts are arranged the collectors *C* for the recovery of zinc-dust. As indicated in Figs. 2 to 7, 90 these collectors are preferably of general cylindrical form, flattened at the sides adjacent to the furnace, and provided with an opening *t*, which registers with the retort-opening *m*, the shortest possible pipe connection 95 or nipple *v* uniting the two openings. The sheet-metal collector is strengthened by a dished bottom *w* and is closed at top by a removable slip cover *x*, adapted, if need be, to receive a quantity of water, so as to regulate 100 the effect, and serving also as a safety-valve should undue pressure develop in the collector. At its lower portion it is provided with a door or slide *z*, covering an opening for the removal of the zinc-dust, and at a point opposite the retort it is provided with a door or slide *z'*, having, as shown, a sight-opening *z''*,

through which the interior of the collector may be observed. When disconnected from the retort, the collector may conveniently be manipulated by means of handles  $x'$ . When 5 in position, it may rest upon any suitable base—as, for instance, the support  $w'$ . The retorts or muffles are charged with the zinc-bearing material from the rear end—i. e., from the end opposite to that at which the collectors are located. At the outset a small sheet-iron cone (indicated in dotted lines in Fig. 2) is attached to the retort-nipple for the purpose of catching the oxid of zinc that is given off at the beginning of the operation. As soon 10 as the color of the deposit at the outer end of the sheet-iron cone indicates the formation of zinc-dust the cone is removed, and slide  $z'$  is closed. The distillation is then continued until the fumes escaping at a small hole  $z^3$  15 (see Fig. 3) near the top of the collector begin to show again the presence of oxid of zinc. The sheet-iron cone or prolong is thereupon again placed in communication with the retort-nipple, so to catch, as in the first 20 instance, the oxid of zinc that is being formed, thereby preventing its admixture with the zinc-dust already collected. The rear end of the retort or muffle is then opened, the spent charge is withdrawn, and the muffle is 25 freshly charged. The operation is then repeated, although, in general, the zinc-dust from each charge is removed from the collector before the fresh charge begins to distil. In so far as the temperature prevailing in the 30 collecting-chamber is concerned we would say that in an ordinary run of eight hours' duration the temperature for about four hours of that period at the region adjacent to the door  $z'$ , is somewhat above the melting-point of 35 zinc (775° Fahrenheit) and thereafter somewhat above the melting-point of lead, (612° Fahrenheit,) although not so high as the melting-point of zinc. During the first four hours the temperature at the upper part of the collector is above the melting-point of lead and below the melting-point of zinc and thereafter somewhat below the melting-point of lead. At the bottom of the collector the temperature during the entire operation is somewhat below the melting-point of lead, although 40 still comparatively high. The size of the collector will depend upon the richness of the charge and the corresponding volume of the zinc-vapors. In practice, we have found that 45 a condenser four feet high and two feet in diameter will collect two hundred and sixty pounds of zinc-dust in twenty-four hours.

In the apparatus shown in Figs. 8 and 9 the retorts or muffles  $n$  are multiplied and are arranged in vertical series, so as to give greater capacity of output, each double vertical series communicating through the openings  $m$  directly with a collecting-chamber  $C'$ , provided with slides  $z^4$  and  $z^5$ , corresponding in 55 function to the slides  $z$  and  $z'$  of the collector  $C$ . At its top each collector  $C'$  is provided with an opening closed by a slip cover or lid

$x^2$ , serving as a safety-valve, said cover having a small aperture  $n'$  of about one inch in diameter for the same purpose as the like aperture  $z^3$  of the collector  $C$ . The furnace is stayed and bonded, as shown, and is provided with the fuel-chamber  $a$ , grate-bars  $b$ , ash-pit  $c$ , arch  $B$ , and chimney-stack  $D$ , as will be readily understood. The mode of operation 70 of this modification of the invention corresponds to that hereinbefore described, the recovery of the zinc-dust taking place in the collectors  $C$ . The prolongs, (one of which is indicated in dotted lines in Fig. 9,) as before, 75 are adjusted to the muffle-openings  $m$  at the outset and toward the end of the operation, so as to catch the oxid-of-zinc vapors developed at those periods, but are of course removed during the period of deposition of the 80 zinc-dust in the collectors. The construction has the advantage of dispensing entirely with the intermediate nipple  $v$  of the collector  $C$ , thereby absolutely insuring against the possibility of the formation of melted zinc at that 85 point. Moreover, it enables one collector to be used for muffles located one above the other, a matter of difficulty if a single sheet-iron collector were employed, because of the fact that in adjusting such sheet-iron collector 90 to the several muffles it is found in practice that it is almost impossible to make the various nipples register exactly with the corresponding openings in the casing and make 95 reliable gas-tight joints.

The recovery of zinc-dust as a by-product in the manufacture of zinc has been heretofore practiced; but the amount thus obtained has borne but a slight ratio to the furnace charge. Our invention, on the contrary, is 105 designed to recover in the form of zinc-dust substantially the entire body of distilled zinc given off from the muffles, a result which has heretofore, so far as we are aware, never been attained or even approximated. The zinc-vapors immediately upon their issuance from the muffle are expanded in the collector while still at the temperature of volatilization and without having an opportunity to liquefy pass at once and in their entirety into the "dust" 110 or granular condition, the product at the prevailing market rates being very much more valuable than either bar-zinc or zinc oxid.

Having thus described our invention, what we claim is—

1. The process of obtaining the substantially maximum yield of zinc-dust or blue powder from a given retort charge, which consists in preliminarily heating the charge to effect the distillation of the zinc, receiving 125 the metallic-zinc vapors given off from the charge, in their substantial entirety from the muffle directly into a collecting-chamber, thereby maintaining their temperature throughout above the point of liquefaction of 130 any substantial portion of the vapor until they have entered the collecting-chamber, and immediately condensing them in said chamber under such conditions of temperature and

expansion as will precipitate them in substantially their entirety in the form of zinc-dust, substantially as described and for the purposes set forth.

5 2. The process of obtaining the substantially maximum yield of zinc-dust or blue powder from a given retort charge, while excluding injurious admixture of zinc oxide therewith, which consists in preliminarily 30 heating the charge to effect the distillation of the zinc, conveying off separately the preliminary oxid-of-zinc vapors generated in the retort, then receiving the metallic-zinc vapors given off from the charge, in their substantial entirety from the muffle directly into a collecting-chamber, thereby maintaining 35 their temperature throughout above the point of liquefaction of any substantial portion of the vapor until they have entered the collecting-chamber, and immediately expanding and condensing them to zinc-dust in said chamber; substantially as described and for the purposes set forth.

20 3. The process of obtaining the substantially maximum yield of zinc-dust or blue powder from a given retort charge, while ex-

cluding injurious admixture of zinc oxide therewith, which consists in preliminarily heating the charge to effect the distillation of the zinc, conveying off separately the preliminary oxid-of-zinc vapors generated in the retort, then receiving the metallic-zinc vapors given off from the charge, in their substantial entirety from the muffle directly into a collecting-chamber, thereby maintaining 40 their temperature throughout above the point of liquefaction of any substantial portion of the vapor until they have entered the collecting-chamber, immediately expanding and condensing them to zinc-dust in said chamber; and interrupting the flow into the collecting-chamber when, at the final stage of the operation, oxid-of-zinc vapors reappear therein; substantially as described.

In testimony whereof we affix our signatures in presence of two witnesses.

GEORGE G. CONVERS.  
ARTHUR B. DE SAULLES.

Witnesses:

OSWIN W. SHELLY,  
EDWARD J. MALLOY.